

## UNITED STATES PATENT OFFICE

2,496,115

## STABILIZATION OF PERFLUORO OILS

William B. Burford, III, Baltimore, Md., and Clifford E. Weber, Schenectady, N. Y., assignors to the United States of America as represented by the United States Atomic Energy Commission

No Drawing. Application February 2, 1948,  
Serial No. 5,894

4 Claims. (Cl. 260—648)

1

This invention relates to the stabilization of perfluoro oils and more particularly to the treatment by means of fluorine of perfluoro oils which are unstable in the presence of fluorine and other vigorous fluorinating agents and which may contain residual hydrogen whereby their stability is improved and the residual hydrogen content thereof is reduced.

Perfluoro oils are a species of perfluorocarbons. Perfluorocarbons are saturated compounds containing only carbon and fluorine. They are chemically inert which makes them particularly useful in applications which involve the handling of fluorine and similar reactive materials. Such perfluorocarbons may be made by passing the vapors of selected hydrocarbons over a bed of cobaltic fluoride. The synthesis of perfluorocarbons is more fully described in the articles by Fowler et al. and Burford et al. which respectively begin on pages 292 and 319 of the March 1947 issue of Industrial and Engineering Chemistry (vol. 39, No. 3). Perfluoro oils are perfluorocarbons which are made by fluorination of petroleum lubricating oils. Such petroleum lubricating oils as well as the perfluoro oils made therefrom contain molecules having from 14 to 21 carbon atoms. Perfluoro oils have average molecular weights varying from 900 to 1100. Assuming a molecular weight of 1000, an arbitrary mean formula of  $C_{20}F_{42}$  may be assigned to these perfluoro oils.

As produced such perfluorocarbons are often associated with small amounts of incompletely fluorinated products which may be designated as hydrofluorocarbons. In the case of a product having a sharp boiling point such as perfluoroheptane, it is feasible to separate it from the hydrofluoroheptanes which may be associated therewith by fractional distillation. However, since perfluoro oils contain molecules having from 14 to 21 carbon atoms they have a boiling range rather than a sharp boiling point. Furthermore, the boiling range of such perfluoro oils overlaps the boiling range of the hydrofluorocarbons that may be associated therewith. Therefore, it is impossible to separate a perfluoro oil from associated hydrofluorocarbons by fractional distillation processes.

It has been found that perfluorocarbons are not chemically inert unless they are rigorously purified. It was discovered that perfluorocarbons would undergo hydrolysis if treated with dilute caustic under mild conditions unless they had been extensively purified by fractionation. Samples of perfluoroheptane and perfluorodimethyl cyclohexane which had a boiling range

2

of only a few tenths of a degree hydrolyzed markedly in comparison with material which had the sharp boiling point of an entirely pure compound. The impurity which caused this reactivity of the perfluorocarbon was assumed to be a trace of incompletely fluorinated material containing hydrogen, but this assumption could not be verified at the time this discovery was made due to the lack of a precise analytical technique for detecting residual hydrogen in the products at that time.

Perfluoro oils find use as coolants, seal liquids and lubricants in mechanical devices used for pumping, storing and disposing of elementary fluorine. It was found that perfluoro oils which had been extensively treated with fluorinating agents and which were therefore assumed to contain no residual hydrogen would consume large amounts of fluorine. This consumption of fluorine eventually resulted in destruction of the oil through a breakdown into very low-boiling fragments and carbon. It was later discovered through the development of improved analytical techniques for detecting hydrogen in perfluoro oils that the oils which were unstable in the presence of fluorine had a residual hydrogen content of the order of a few tenths of 1% by weight. However, the marked chemical reactivity of these perfluoro oils toward fluorine was entirely out of proportion to their residual hydrogen content.

In order that perfluoro oils might continue to be used in devices for handling elementary fluorine, it was necessary to devise a method of stabilizing these oils so that they would not be reactive with fluorine. Attempts to stabilize these perfluoro oils by repeatedly treating them with solid cobaltic fluoride at 200° to 250° C. were unsuccessful. Oils so treated were still very reactive to fluorine although they were not quite as reactive as perfluoro oils that had not been so treated. Oils treated with cobaltic fluoride had a useful life about four times as long as oils that had not been so treated but they were still not wholly satisfactory since they were no longer usable after a period of two months. It was also discovered that perfluoro oils which had been treated with fluorine at any fixed temperature were also still fairly reactive to fluorine.

It is, therefore, an object of the present invention to devise a method of stabilizing perfluoro oils so that such oils will not be reactive with fluorine and other vigorous fluorinating agents. A further object of the present invention is to treat perfluoro oils so as to remove

therefrom any residual impurities, such as hydrogen which may be causing said oils to be reactive with fluorine. A still further object is to produce fluorinated lubricating oils that are not unstable in the presence of fluorine and other vigorous fluorinating agents. Another object is to produce stable perfluoro oils by a simple and efficacious procedure. Other objects will appear hereinafter.

These objects are accomplished in accordance with the present invention in which perfluorocarbon materials, such as fluorinated lubricating oils having an approximate formula,  $C_{20}F_{42}$ , are rendered relatively inert to elementary fluorine by treatment with the latter material under controlled conditions. The treatment employs fluorine in concentrations up to 50%, but preferably about 20% mixed with a suitable diluent, such as dry nitrogen. This mixture of gases is bubbled through the liquid perfluoro oil at a suitable rate in a simple tubular reactor which may be heated and may or may not be equipped for stirring. Reactive anhydrous catalysts such as cobaltic fluoride ( $CoF_3$ ), manganese trifluoride ( $MnF_3$ ), or ceric fluoride ( $CeF_4$ ) may be present, if desired, in amounts of the order of 2% to 10% by weight of the perfluoro oil. The essential feature of the treatment is to complete the reaction between the fluorinated oil and the fluorine at each of several temperatures in an increasing scale beginning at a relatively low value in the range from 60° to 150° C. This may be accomplished by treating with fluorine at a fixed temperature until analysis of the gases leaving the reactor shows that very little fluorine is being absorbed, after which the temperature is slightly increased and treatment with fluorine continued until analysis of the exit gases again shows that little fluorine is being absorbed in the reactor, and so on. Since the absorption of fluorine is temperature dependent, the following alternative procedure is also expedient. The exit gases from the reactor may be analysed at frequent intervals, and the temperature slowly raised at treatment with fluorine proceeds in such a manner as to maintain the percent of fluorine absorbed at any convenient value less than 100%, such as 80-95%. This alternative procedure is somewhat more convenient in operation and results in equally good stabilization but with a slightly reduced yield. In accordance with another modified procedure, the temperature throughout the fluorine treatment is maintained high enough so that essentially all of the fluorine is being absorbed by the fluorinated lubricating oil, and the concentration of fluorine in the exit gases approximates 20 to 30 parts per million. Fluorine treatment and the concomitant upward adjustment of temperature is continued until as high a temperature of treatment as possible is reached. This is usually determined by the boiling point of the liquid being treated, and in the case of perfluoro oils having an approximate formula,  $C_{20}F_{42}$ , this terminal temperature is about 300° C. The treatment is considered complete when the fluorine absorption at the highest temperature of treatment is of the order of 3% to 6% of the fluorine being fed to the reactor.

Fluorinated lubricating oils which have been so treated absorb very little fluorine at temperatures below their final treatment temperature and have a low hydrogen content (less than 0.001% by weight). They may be used in contact with fluorine and similar corrosive gases with very much

less cracking and degradation than is possible with fluorinated lubricating oils that have not been subjected to the stabilizing treatments of the present invention. Available test methods indicate that perfluoro oils which have undergone stabilization by this method are many times more stable to the action of elementary fluorine and similar fluorinating agents. For example, a perfluoro oil having a very low hydrogen content which has not undergone stabilization will absorb all fluorine supplied to it at temperatures as low as 200° C., whereas the same oil, when stabilized in accordance with the present invention, will absorb only from 3% to 7% of the fluorine supplied to it at 300° C.

In order that the invention may be more fully understood the following detailed examples are given to illustrate it. It is to be understood that these examples merely illustrate but do not limit the present invention.

#### EXAMPLE I

700 parts by volume of a perfluoro oil containing 0.073% of hydrogen were placed in a copper cylinder which served as a reactor. This reactor was provided with an electrical heater, a stirrer and a fluorine inlet at the bottom which was covered by a 100-mesh copper screen. Fluorine diluted with nitrogen to a fluorine concentration of 20% was passed into the reactor at a rate of 1000 parts by volume per minute. The temperature of the reactor was maintained at 150° C. during the first 2 hours of treatment and then raised to 200° C. for the next 4.4 hours of treatment. During the next period of 3 hours the temperature was held at 250° C., and finally the temperature was maintained at 300° C. for the last period of treatment for 3 hours. A 78% yield of a stabilized perfluoro oil was obtained which showed very little tendency to absorb fluorine at 300° C. The stabilized oil had a lighter color than the oil which had not been stabilized by the treatment with fluorine.

The unstabilized perfluoro oil mentioned in the preceding paragraph could not be successfully stabilized by treating it at a constant fixed temperature of 150° C. with 20% or 40% fluorine supplied at a flow rate of 5 units of volume of gas per minute to each 3 units of volume of oil in the reactor. Even after from four to six hours of treatment with fluorine, the treated oil retained the property of absorbing over 80% of the fluorine supplied thereto at 250° C. This showed that stabilization of this oil cannot be satisfactorily accomplished by treating it with fluorine at a constant fixed temperature.

#### EXAMPLE II

Unstabilized perfluoro oil which contained less than 0.06% of hydrogen was treated with fluorine in a copper cylinder which was electrically heated and equipped with a stirrer and to which fluorine was admitted through a 100 mesh copper screen in its lower end. In a series of seven runs 18% fluorine was passed into the reactor at a flow rate equal to 1.6 units of volume of gas per unit volume of perfluoro oil in the reactor per minute. The temperature was held at 150° C. for two to three hours, then maintained for two hours at 200° C., for one hour at 250° C., and finally held for two to three hours at 280° C. The total treatment time varied between eight and twelve hours

with no appreciable change in the yields. The average yield on these seven runs was 86% with a low yield of 80% and a high yield of 90%. The product had a very low degree of ability to absorb fluorine compared with the unstabilized oil from which it was prepared. The stabilized oil has a viscosity of 58.2 seconds Saybolt (about 19 centipoises) at 210° F., whereas the unstabilized oil from which it was prepared had a viscosity of 65.8 seconds Saybolt (about 23 centipoises) at 210° F. The unstabilized oil had a reflux boiling point at a pressure of 10 mm. of 155° C., whereas the stabilized oil made in accordance with this example had a reflux boiling point of 140° C. at a pressure of 10 mm. The yields in this example are better than in the preceding example because of slight improvements made in the apparatus and operating technique.

#### EXAMPLE III

700 parts by volume of a perfluoro oil containing 0.073% of hydrogen were placed in a reactor such as that described in Example I. To the oil was added anhydrous cobaltous fluoride ( $\text{CoF}_2$ ) in an amount equivalent to 5% of the weight of the oil. The reactor was brought to a temperature of 150° C. and held there for two hours while the reactants were stirred and 20% fluorine was passed into the reactor at a rate of 1000 parts by volume per minute. Then the temperature of the reactor was increased to 200° C. and held there for four hours while stirring and the introduction of fluorine were continued. The temperature was then raised to 250° C., and held there for three hours and finally raised to 300° C. and held there for three hours while continuing the introduction of 20% fluorine to the reactor at the rate of 1000 parts by volume per minute. A 90% yield of a stabilized perfluoro oil which had a very slight tendency to absorb fluorine at 300° C. was obtained. Much of the cobaltous fluoride in the reactor was converted to cobaltic fluoride by reaction with fluorine. The reactor used in this example and the perfluoro oil treated were the same as in Example I. The conditions of treatment were substantially the same except for the employment of cobalt fluoride as a catalyst. It will be seen by comparing this example with Example I that the use of cobalt fluoride as a catalyst results in a somewhat better yield than was obtained when no catalyst was present.

#### EXAMPLE IV

A number of treatments of an unstabilized perfluoro oil which contained less than 0.06% of residual hydrogen were carried out by supplying fluorine thereto under the conditions indicated in the following table. In the following table "Fluorine flow rate" designates the number of units of volume of diluted fluorine gas passed into a unit volume of perfluoro oil per minute. "Fluorine concentration" gives the percent by volume of fluorine in the fluorine-dry nitrogen mixtures. The "Time in hours" indicates the number of hours the perfluoro oil was subjected to fluorine treatment. In all ten hour runs the oil was treated with fluorine at 150° C. for three hours, at 200° C. for two hours, then at 250° C. for two hours, and finally at 280° C. for three hours. In all five hour runs the time of treatment at each temperature was halved. In each run the temperature at the termination of the

treatment was 280° C. Under "Catalyst" the per cent indicates the ratio of the weight of catalyst to the weight of perfluoro oil being treated.

TABLE I

| Run | Fluorine Concentration | Fluorine Flow Rate | Time  | Catalyst            | Crude Yield |
|-----|------------------------|--------------------|-------|---------------------|-------------|
| 10  | Per cent               |                    | Hours |                     | Per cent    |
| A   | 18                     | 1.4                | 10    | None                | 85          |
| B   | 18                     | 1.4                | 10    | 3.5% $\text{CoF}_2$ | 95          |
| C   | 37                     | 1.4                | 5     | None                | 93          |
| D   | 38                     | 2.9                | 5     | do                  | 92          |
| E   | 38                     | 2.9                | 5     | 3.5% $\text{CoF}_2$ | 94          |
| F   | 37                     | 2.9                | 3.5   | None                | 91          |

The products obtained in all of these runs exhibited very little capability of absorbing fluorine at 300° C. and hence were adequately stabilized.

- 20 The use of cobalt fluoride as a catalyst appeared to improve the yields. The use of as high a flow rate as possible which does not cause the perfluoro oil to be carried out of the treatment apparatus due to misting was found to be desirable. 25 Furthermore, it was found that fluorine should be used in as high a concentration as will not cause charring or degradation of the perfluoro oil in order to decrease the time of treatment.

#### EXAMPLE V

One of the alternate methods of stabilizing perfluoro oils in accordance with the present invention is to start the fluorine treatment at about 35 150° C., and to maintain a constant absorption of fluorine by variation of the treatment temperature. Thus a gradual increase of temperature permits the maintenance of a fixed rate of absorption of fluorine. The following table gives 40 the data on a number of stabilization runs made on a perfluoro oil having a residual hydrogen content of 0.1% and composed of molecules having an average of 20 carbon atoms. These runs were conducted so that substantially 100% of the 45 fluorine was absorbed except in the final part of the treatment. The runs were each started at a temperature high enough to cause 100% absorption of fluorine, the minimum 100% absorption temperature was found at once, and the 50 temperature of treatment slowly increased to maintain 100% fluorine absorption until the maximum temperature (usually 300° C.) was reached. After reaching the maximum temperature, the 55 fluorine absorption decreased slowly with continued treatment. The run was terminated when the fluorine absorption had become 10% or less as shown by analysis of the exit gases from the reactor. The 100% absorption was followed and maintained by testing the exhaust gases with 60 moist potassium iodide paper.

In the following table "Fluorine flow rate" designates the number of units of volume of diluted fluorine gas passed into a unit volume of perfluoro oil in the reactor per minute. The "Time in hours" designates the number of hours the perfluoro oil is subjected to fluorine treatment. The "Termination temperature" indicates the highest temperature to which the perfluoro oil 70 was heated before the fluorination treatment was ended. Under "Catalyst" the per cent indicates the ratio of the weight of catalyst to the weight of perfluoro oil being treated. "Fluorine concentration" gives the per cent by volume of fluorine in the fluorine-nitrogen gas mixture.

7  
Table 2

| Run | Fluorine Concentration | Fluorine Flow Rate | Time  | Termination Temperature | Catalyst              | Crude Yield |
|-----|------------------------|--------------------|-------|-------------------------|-----------------------|-------------|
|     | Per cent               |                    | Hours | °C.                     |                       | Per cent    |
| x-1 | 18                     | 1.7                | 6.75  | 300                     | None                  | 81          |
| x-2 | 37                     | 1.7                | 5.75  | 276                     | do                    | 87          |
| x-3 | 37                     | 1.7                | 5.5   | 300                     | do                    | 87          |
| x-4 | 18                     | 3.3                | 5.5   | 300                     | do                    | 81          |
| x-5 | 18                     | 1.7                | 13.5  | 250                     | 3.2% CoF <sub>3</sub> | 87          |
| x-6 | 18                     | 1.7                | 6.75  | 300                     | None                  | 81          |
| x-7 | 18                     | 6.7                | 3     | 300                     | None                  | 81          |

In all of the above runs it was noted that for each 300 cubic centimeters of perfluoro oil being treated from 1.2 to 1.7 mols of fluorine were absorbed. The runs with 18% fluorine required the longest treatment time and, while the yields of stabilized oil were poorer, the product had a somewhat better stability toward fluorine than products secured in some of the other runs. The one run (x-4) made with 18% fluorine at twice the normal flow rate gave a better yield of a product of very slightly inferior stability to fluorine than the products made at the normal flow rate. The runs with 37% fluorine were made in somewhat less than the total time required for treatment with 18% fluorine at the 1.7 flow rate and resulted in greater yields of products which were but slightly less stable to fluorine than the products stabilized with 18% fluorine at the 1.7 flow rate. All of the runs described in the above table were carried out in a small reactor which consistently gave smaller yields than the reactors used in obtaining the results which were described in the other examples of this application.

Attempts to stabilize the same perfluoro oil used in the runs recorded in Table 2 above by treating it for about 6 hours at a fixed temperature of 150° C. with 20% or 40% fluorine passed into the oil at a flow rate of 1.7 unit volumes of gas per unit volume of oil per minute resulted in an unstabilized product which absorbed more than two thirds of the fluorine supplied thereto at 250° C. Two more attempts were made to stabilize this same perfluoro oil by treating it for about 12 hours at a fixed temperature of 300° C. with 20% and 40% fluorine. After 12 hours of treatment with 20% fluorine a crude yield of only 52% was obtained, and the product was unsatisfactorily stabilized since it absorbed 25% of the fluorine supplied thereto at 250° C. After 14 hours of treatment with 40% fluorine almost no perfluoro oil was left in the reactor. These attempts to stabilize perfluoro oils at single fixed temperatures showed that, at moderate temperatures, treatment with fluorine yielded products which were essentially unstabilized and capable of readily absorbing much more fluorine at higher temperatures while treatment at higher temperatures resulted in low yields of products that still possessed a high capacity to absorb fluorine. In other words, satisfactory stabilization of an unstabilized perfluoro oil cannot be attained by treating it with fluorine at a single fixed temperature.

Yield data in the above examples are calculated on a basis of the ratio of the amount of specification grade oil charged to the reactor to the amount of specification grade oil recovered from the reactor after the treatment is complete. The yields using perfluoro oils containing 0.1% or less of residual hydrogen generally vary from 80% to 95%.

The preferred apparatus used for treating per-

fluoro oils with fluorine comprises a copper or monel tube equipped with a heating jacket, thermocouple well and a motor driven, paddle-shaped stirrer. At the bottom of the tube where the fluorine enters a 100 mesh bronze screen is placed across the interior opening. This screen disperses the entering fluorine to prevent any effect similar to ignition at a jet. In operation, the unit is filled nearly full of perfluoro oil to be treated, and diluted fluorine gas is bubbled through it at a suitable flow rate. The exit gases from the reactor unit pass through a reflux condenser or mist trap and thence to a gas sampling manifold before being vented to a disposal unit.

The fluorine concentration in the exit gases was conveniently followed by an analysis based upon the liberation of iodine from a potassium iodide solution followed by titration with a standard thiosulfate solution. The gas was sampled in calibrated glass bulbs, after which fluorine was absorbed by admitting a potassium iodide solution.

From the data obtained it appears that stabilization of a perfluoro oil with fluorine is promoted by the following factors: (1) intimate contact between the fluorine and perfluoro oil achieved by rapid and highly efficient stirring; (2) high flow rate of gas; (3) moderate fluorine concentration in the gas, and (4) the presence of catalytic proportions of cobalt fluoride in the reactor. Careful attention to these factors results in better yields, higher stability characteristics of the products, and completion of the reaction in the shortest possible period of time. It was also noted that better yields were obtained if the fluorine absorption was near 100% throughout the run resulting in the shortest possible time of treatment, and if the temperature was smoothly increased to the highest possible value, 285°-315° C., which was determined by the boiling point of the oil and the characteristics of the reactor. If the temperature was too high, particularly during the early stages of the run the yield was decreased, and if the run were extended by holding the temperature too low, the yield fell off due to cracking.

It has been found that stirring greatly facilitates the absorption of fluorine by unstabilized perfluoro oils. In one reactor it was found that at 150° C. the fluorine absorption was 33% when the stirrer stood idle but that 83% of the fluorine being passed into the oil was absorbed when the stirrer was operated at 1200 R. P. M. In another reactor it was noted that at 100° C. only 0.5% of the fluorine was being absorbed when the stirrer stood idle but that 61% of the fluorine was absorbed when the stirrer was rotated at 600 R. P. M. and 83% of the fluorine was being absorbed when the stirrer was rotated at 1200 R. P. M.

The optimum flow rate for fluorine depends both upon the design of the treatment apparatus and upon the concentration of the fluorine. For a given treatment system, the optimum concentration of fluorine and flow rate must be experimentally determined to give the best possible yield in the shortest treatment time. Obviously, a high flow rate of fluorine which causes excessive losses of perfluoro oil from the treatment system due to misting is to be avoided. If the fluorine concentration is held down to about 20% the flow rate may be as high as is feasible provided no perfluoro oil is being entrained from the reactor in the form of mist. Flow rates varying from 1 to 7 units of volume of diluted fluorine gas per

unit of volume of perfluoro oil in the reactor per minute have been found to be feasible. However, flow rates of about 3 to 4 units of volume of diluted fluorine gas per unit of volume of perfluoro oil per minute appear to be optimum. Flow rates greater than this are inadvisable with 37% fluorine if degradation of the oil is to be avoided.

The fluorine used in the reaction is diluted with an inert gas such as nitrogen to cut down the vigor of the ensuing reaction. Fluorine concentrations varying from 5% to 50% may be employed, but, as indicated in the preceding paragraph, it is inadvisable to employ high fluorine concentrations when the diluted fluorine gas is flowing into the reactor at a high flow rate, if degradation of the perfluoro oil being treated is to be avoided. In many reactors it was found that a fluorine concentration of about 20% gave the best yields.

It was found that the use of catalytic proportions—2 to 10% based upon the weight of perfluoro oil being treated—of cobalt fluoride tended to increase the yield and quality of the stabilized perfluoro oil produced. In one set of reactors the best yield obtained without the use of cobaltic fluoride was 88% compared to 93% with catalyst present, while 98% of the recovered charge boiled in the proper range when cobaltic fluoride was used, compared to 90 to 96% without a catalyst. The cobalt fluoride is added to the reactor in the form of anhydrous cobaltous fluoride and is converted in situ to cobaltic fluoride by reaction with fluorine. Manganic fluoride ( $MnF_3$ ) or ceric fluoride ( $CeF_4$ ) may be used in place of cobaltic fluoride as a catalyst. Manganese fluoride is added to the reactor as anhydrous manganous fluoride ( $MnF_2$ ) and converted in situ to manganic fluoride by fluorine. Similarly, anhydrous cerous fluoride ( $CeF_3$ ) is added to the reactor and converted in situ to ceric fluoride.

Stabilized perfluoro oil from a physical point of view is practically identical with unstabilized perfluoro oil except for the removal of any color present in the starting material. The identical distillation fractions before and after stabilization are surprisingly alike. Since variations in physical properties are minor, the stabilization process herein described can be readily adapted to perfluoro oils meeting certain desirable physical specifications and will not cause changes which result in a large proportion of the stabilized perfluoro oil having properties which lie outside of the desirable specifications of the untreated perfluoro oil.

The chief chemical reaction which takes place during the stabilization treatment appears to be the replacement of residual hydrogen with fluorine. However, it is entirely possible that other reactions such as removal of double bonds and isomerization or other changes in molecular configuration lead to the formation of molecules that are no longer reactive with fluorine.

As can be seen, in accordance with the present invention, a method has been developed that leads to stabilization of perfluoro oils toward fluorine gas and other vigorous fluorinating agents. This method comprises treatment of the perfluoro oil with dilute fluorine at slowly increasing temperatures up to the boiling point of the oil. Such treated perfluoro oils show a marked stability toward elementary fluorine and will react only slightly at elevated temperatures

in the neighborhood of 300° C. Yields are good averaging 88% or better. The removal of hydrogen appears to accompany the process of stabilization and may be the basis of this phenomenon. Many of the untreated oils which contain approximately 0.02% of residual hydrogen are found after the stabilization treatment to contain 0.001% or less of residual hydrogen.

Resort may be had to such modifications and variations as fall within the spirit of the invention and the scope of the appended claims.

We claim:

1. The process of stabilizing and removing chemically combined residual hydrogen from a perfluoro oil containing less than 1% of residual hydrogen which comprises subjecting said perfluoro oil to treatment with fluorine at a series of increasing temperatures from a base starting range of 60° to 150° C. to a maximum temperature lying between 250° C. and 315° C.

2. A process as recited in claim 1 which is carried out in the presence of an anhydrous catalyst selected from the group consisting of cobaltic fluoride, ceric fluoride and manganic fluoride.

3. The process of stabilizing and removing chemically combined residual hydrogen from a perfluoro oil containing less than 1% of residual hydrogen which comprises passing diluted fluorine gas through said perfluoro oil at a base starting temperature lying in the range of 60° to 150° C., increasing the temperature by an increment of several degrees centigrade when it is found that little fluorine is being absorbed by the perfluoro oil, making at least one more further stepwise increase in the temperature of treatment when it is again found that the perfluoro oil is absorbing little fluorine, said stepwise increase in the temperature of treatment being continued until final treatment temperature lying between 250° C. and 315° C. has been attained, and continuing the treatment with diluted fluorine at the final treatment temperature until very little fluorine is being absorbed by the perfluoro oil.

4. The process of stabilizing and removing chemically combined residual hydrogen from a perfluoro oil containing less than 1% of residual hydrogen which comprises passing diluted fluorine gas through said perfluoro oil at a base starting temperature lying in the range of 60° to 150° C., gradually increasing the temperature so that the fluorine absorption is substantially continuous, terminating the treatment with diluted fluorine at a temperature lying between 250° C. and 315° C. when the perfluoro oil is absorbing 10% or less of the fluorine supplied thereto at the final treatment temperature.

WILLIAM B. BURFORD, III.  
CLIFFORD E. WEBER.

#### REFERENCES CITED

The following references are of record in the file of this patent:

#### UNITED STATES PATENTS

| Number    | Name                   | Date          |
|-----------|------------------------|---------------|
| 2,013,030 | Calcott et al. -----   | Sept. 3, 1935 |
| 2,446,251 | Stricklin et al. ----- | Aug. 3, 1948  |

#### OTHER REFERENCES

Struve et al., Ind. Eng. Chem., vol. 39, 352-4 (1947).